

## UNITED STATES PATENT OFFICE

2,196,788

NONBLEEDING BLUE PRINT AND PROCESS  
OF MAKING THE SAME

Harold J. Brunk, Chicago, and Morris Dickason,  
Oak Park, Ill., assignors to The C. F. Pease  
Company, Chicago, Ill., a corporation of Dela-  
ware

No Drawing. Application July 29, 1937,  
Serial No. 156,412

2 Claims. (Cl. 95—6)

This invention relates to photoprints and an improved process of making the same, and more particularly to a process whereby "bleeding" of the photoprints may be prevented.

- 5 The usual process of blueprinting consists of applying a light sensitive coating to paper or a like material, exposing the paper to a light with a tracing or negative between the light source and the coated side of the paper and thereafter developing the coated paper to produce a blue sheet with white lines or a white sheet with blue lines.
- 10 The coating ordinarily used consists of a mixture of potassium ferricyanide and an organic salt of iron such as ferric ammonium oxalate, and is applied by means of an aqueous solution of the mixture. Upon exposure to light the potassium ferricyanide and the ferric ammonium oxalate are partially reduced to potassium ferrocyanide and ferrous ammonium oxalate, respectively.
- 15 20 When the paper is washed with water the reduced chemicals react with the unreduced to produce the insoluble blue compounds known as Turnbull's blue and Prussian blue. The unexposed chemicals as well as the excess of the unreduced compounds, being soluble, are washed away, leaving blue lines or areas in the exposed portions.

- 25 Great difficulties, however, are encountered in attempting to produce a sharp line of demarcation between the exposed and unexposed portions. When the water is applied to "fix" the exposed chemicals and wash off the soluble substances it causes the occurrence of what is known as bleeding. The unreduced chemicals of the exposed portion dissolve in the water and thus react with the reduced ferricyanide and ferric salt of the same area to form the essential insoluble blue substances. However, before this reaction is complete some of the reduced chemicals are carried 30 by the water into the unexposed portions of the paper thereby forming insoluble blue compounds on the edge of the unexposed portions of the paper, producing a ragged line or other unsightly irregularities.

- 35 40 45 50 55 Various processes have been devised to prevent bleeding but the present invention has certain advantages over the same.

- One feature of our invention is the prevention of bleeding and thus the production of photoprints having clearly defined lines. Another feature is an increase in the speed at which the printing may be carried on. Another feature is the development of a process in which the printing may be carried on at a constant speed regardless of the concentrations of the sensitizing

agents used. Still another feature is the production of a more uniform color than has been possible heretofore. Other features and advantages will be apparent from the following description of our invention.

We have found that pure potassium ferricyanide, although sensitive to light when mixed with a light sensitive ferric salt, is practically completely unaffected by light when not so mixed. Certain ferric salts, such as ferric ammonium oxalate, for example, are, on the other hand, very easily reduced by light. In fact, the ferric salts are more sensitive to light when used alone than when mixed with the ferricyanide as in the usual blue print process. Potassium ferricyanide reacts with ferrous compounds (which are formed by the reduction of ferric salts) to form ferrous ferricyanide, a water-insoluble blue substance known as Turnbull's blue. Thus, if the paper to be printed is coated first with a light sensitive ferric salt and then with a ferricyanide of an alkali metal and thereafter exposed to light the paper need only be washed to produce a well colored non-bleeding blue print. The ferricyanide, which is unaffected by the light, reacts with the exposed reduced ferric salts to form ferrous ferricyanide (Turnbull's blue) which is insoluble and does not run or bleed.

Also, where the two layers meet there occurs, to a certain extent, a mixing of the ferricyanide and the ferric salt. As a result, at this interface both compounds are at least partially reduced upon exposure. Washing with water thus causes an additional reaction, to wit—the reaction between the ferrocyanide and the unreduced ferric salt to form ferric ferrocyanide (Prussian blue) which is also insoluble. Prussian blue is deep blue in color and, though present only in a small amount, serves to deepen and improve the color of the print. On the unexposed portions the ferric salts and the ferricyanide, being water soluble, are washed away leaving a white background.

The first layer of the coating may be composed of any light sensitive ferric salt. Among the compounds which have been found particularly satisfactory are ferric ammonium oxalate, ferric ammonium citrate, ferric chloride, ferric oxalate, ferric potassium oxalate, ferric sodium oxalate, ferric ammonium chloride, ferric ammonium sulfate, and ferric ammonium tartrate.

55 The salt may be applied to the paper or like material in any convenient manner. A uniform coating which adheres firmly to the paper may be obtained by applying an aqueous solution of the salt either by dipping, spraying, or by passing

the paper over a roller which is so mounted as to dip in the solution. If, as we prefer, the last method is used, it is usually desirable to use a resilient roller and rotate the roller in the opposite direction to that in which the paper is moving. In this way the surface of the paper is roughened slightly and the solution penetrates more deeply into the surface of the paper. As a result, the salt and, after the process is completed, the coloring material adheres more firmly to the surface of the paper.

The concentration of the ferric salt solution may vary over a wide range. Any quantity between a few percent and saturation may be used with satisfactory results. After application the solution should be allowed the same time to soak into the paper and to dry as is used with the ordinary blue printing solutions.

The upper or second layer of the coating, which may be applied as soon as the first layer is dry, consists of a ferricyanide compound preferably of an alkali metal such as potassium. This coating also may be applied in any convenient manner. The application of a solution of the compound is usually found to be the simplest and best method of coating. We prefer to apply this solution to the paper by means of a roller which dips into the solution. We have found that in using rollers to apply the solution it is advantageous to rotate the roller in the same direction as that of the movement of the paper. A more even coating and less contamination of the upper layer with the ferric salts of the lower layer results. Also, pin spot defects, caused by failure of the coating to cover certain small portions of the paper, are eliminated if this trouble is not inherent in the paper stock. If it is desired to make the paper completely bleedproof, it is usually preferable to use two successive rollers to apply the second layer. In this way a heavier but still uniform coating is obtained.

In using a roller to apply the coating to the paper, the rate of travel of the paper and the surface speed of the roller may be adjusted so that the desired amount of solution will be picked up by said roller and applied as an even coating and at a rapid rate. In the coating of blue print paper as now practiced, an excess of the coating solution is usually applied, which excess is then removed by compressed air or by a scraper.

Before the paper is rolled up for storage, the second roller should be perfectly dry. The drying process may be speeded up by the use of an air blast or other convenient means. If the paper is not completely dry it should be printed within a day or two of the coating since it will deteriorate quite rapidly.

We have found that this second coating is particularly valuable when used over the under coating described herein. Although it may be used over the ordinary blue print sensitizing agent consisting of a ferric salt and a ferricyanide, nevertheless in such a case it will tend to cut down the color and slow up the printing. Hence this second coating should preferably be applied over a coating consisting of a ferric salt or salts alone.

The concentration of the ferricyanide solution used should preferably be below ten percent. Usually it is desirable to use between one percent and six percent depending upon the concentration of ferric salt used in the first coating. We have found that a ferricyanide concentration of approximately one-fifth that of the concentration of the ferric salt is particularly satisfactory.

The paper containing the dry two-layer coating is exposed to light through a negative or other tracing. The light does not affect the outer coating of ferricyanide but does reduce the exposed portions of the under coating of ferric salt, and at the interface between the two layers, where the ferricyanide and the ferric salt are mixed, both are reduced. Either sunlight or artificial light may be used to effect the reduction.

The paper undergoes a distinctive color change as exposure takes place. From the light yellow of the unexposed sensitized paper the change is to light blue and blue grey at complete exposure with increasing greying at overexposure. The operator of the process is thus enabled to follow closely the reaction which occurs.

With our process a satisfactory color over a wider range of exposures is possible. Perhaps this is the result of the greater sensitivity to light of the ferric salts alone as compared with the ordinary blue print coating, but at any rate the exact control of exposure which has heretofore been necessary in blue printing is no longer required.

The printing speed may be kept constant regardless of the concentrations of the two solutions by which the coatings are applied. This is a distinct advantage since in the ordinary process the greater the proportion of ferricyanide used in the coating, the slower is the reduction upon exposure to light and hence the slower is the printing speed which must be used.

Upon washing the exposed paper with water, the reduced ferric salts on the exposed portions are fixed by reaction with ferricyanide of the outer layer to form insoluble blue salts, while the unreduced salts on the unexposed portions, being soluble, are washed away leaving a white background. Similarly at the interface where both the ferricyanide and the ferric salt have been reduced, Prussian blue is formed by the reaction of the ferrocyanide and the unreduced ferric salt.

Since the ferricyanide is distributed over the ferrous salt it is dissolved by the water first and reacts to form the insoluble Turnbull's blue before the ferrous salt can be washed into the unexposed portions to cause bleeding.

The following equations represent what are probably the principal types of reaction occurring:



The ferrous ferricyanide is a water insoluble blue salt known as Turnbull's blue. It serves to color the exposed portions of the photoprint and by its precipitation prevents the running of any of the ferrous salt into the unexposed portions. The ferric ferro-cyanide, also insoluble, although present only in a small quantity aids in producing a deeper color. Thus, the unexposed portions are covered with the ferric salt and the ferricyanide. Since both of these compounds are soluble they are washed away by the water, and bleeding is prevented.

Instead of applying the two coatings before exposure it is possible to apply only the ferric salt coating before exposure and then after exposure wash the paper with a solution of a ferricyanide to fix the reduced ferric salt. By this process a bleedproof paper is obtained. However, we prefer to use two dry coatings before

exposure since a small amount of Prussian blue, which produces a desirable color, is formed, and in general more satisfactory results are obtained in this way. Also a step in the actual printing process, the application of a ferricyanide solution, is eliminated with a resultant saving in printing time and equipment.

It is often desirable to have a very white background in the blue print. If so, certain bleaching agents may be incorporated in one of the layers of the coating, preferably the outer or ferricyanide layer, when the paper is being sensitized. Among the substances which are suitable for this purpose are alkali metal oxalates, 10 tartrates, and phosphates.

Although our invention has been described in connection with so called blue prints, it may be used as well with any photoprinting process on a fibrous sheet or on any other suitable material which will serve the same purpose. Also, 20 although certain reactions and equations have been used to illustrate the invention, we do not wish to be limited thereto.

We claim:

25 1. A method of making nonbleeding photo-prints which comprises applying to paper, with

a resilient roller, a solution of ferric ammonium oxalate, the roller being rotated in the direction opposite to the movement of the paper, allowing said solution to dry, and then applying with at least one roller a solution of potassium ferricyanide to form a second coating, the roller being rotated in the direction of the movement of the paper, exposing portions of the coated paper to light to reduce the ferric compound on these portions, and thereafter washing the paper with 10 water whereby insoluble iron compounds are formed on the exposed portions and the soluble salts are washed off the unexposed portions.

2. A method of making nonbleeding photo-prints which comprises applying to a sheet material a coating of a solution of a light sensitive salt of iron by means of a roller, said roller being rotated in the direction opposite to the movement of the sheet material, allowing said coating to dry, then applying with a roller a solution of a 15 ferricyanide of an alkali metal to form a second coating, said last mentioned roller being rotated in the direction of the movement of the sheet material, and allowing the second coating to dry. 20

HAROLD J. BRUNK. 25  
MORRIS DICKASON.